

# United States Patent Office

2,980,611

Patented Apr. 18, 1961

1

2,980,611

# SILICA-THICKENED GREASE CONTAINING ACID AMIDE DISPERSANT

Thomas W. Martinek and Ernest F. Fronczak, Crystal Lake, Ill., and Nathaniel L. Remes, Miami, Fla., assignors to The Pure Oil Company, Chicago, Ill., a corporation of Ohio

No Drawing. Filed Dec. 24, 1957, Ser. No. 704,893

**20 Claims. (Cl. 252—28)**

This invention relates to new and useful improvements in grease compositions, and more particularly to a silica-thickened grease utilizing an improved dispersant for the silica gelling agent.

This invention is based upon our discovery that acid amides are superior dispersants for silica-thickened greases. This invention is further based upon our discovery that certain of the acid amides are not only useful as dispersants for silica-thickened greases but are also water-proofing agents which resist destruction of the grease upon contact with water.

Although the classical definition of lubricating greases is restricted to oils which are thickened or gelled with soaps, there has been developed a number of grease-like lubricants which are based upon synthetic lubricating liquids other than oil, or which utilize gelling or thickening agents other than soaps, but which are recognized as greases. In fact, non-soap-thickened greases have been given considerable attention in recent years for high temperature applications, since these greases do not melt at elevated temperatures. These greases are discussed at considerable length in "Manufacture and Application of Lubricating Greases," Boner, Reinhold (1954). The non-soap-thickened greases differ very substantially from the soap-thickened greases and differ among themselves to a very great extent. For example, the non-soap-thickened greases generally are less susceptible to bleeding and to change of consistency on increase of temperature. Bentone greases are thermally stable and mildly resistant to water. On the other hand, silica-thickened greases are thermally stable but decompose readily upon contact with water unless waterproofing agents are used to prevent separation of the silica particles from the oil. Additives which are used for various purposes in connection with the soap-thickened greases are quite variable in their effect on the various non-soap-thickened greases. For example, metal carbamates and thiocarbamates which are reported (in U.S. Patents 2,652,362 and 2,652,363) to be useful as corrosion inhibitors and stabilizers for soap-thickened greases are completely ineffective as stabilizers or dispersants for bentone and silica-thickened greases. Butyl stearate and coconut oil are each reported (in U.S. Patent 2,662,058) to be useful as dispersion aids for bentone greases but have been found to be completely ineffective as dispersants for silica-thickened greases. These variations in the effect of stabilizers and dispersants for soap-thickened and non-soap-thickened greases indicate the highly empirical nature of the grease-making art in general and the art of making non-soap-thickened greases in particular.

It is therefore one object of this invention to provide a new and improved silica-thickened grease of high yield.

Another object of this invention is to provide a new and improved silica-thickened grease containing a dispersant for the silica which also prevents decomposition of the grease upon contact with water.

A feature of this invention is the provision of an improved silica-thickened grease which utilizes oil-soluble acid amides as dispersants.

Another feature of this invention is the provision of an improved silica-thickened grease which utilizes oil-

2

soluble, water-insoluble acid amides as dispersants for the silica, which amides also function to stabilize the grease structure against water.

5 Other objects and features of this invention will become apparent from time to time throughout the specification and claims as hereinafter related.

In carrying out this invention, silica-thickened greases are prepared by dispersing in a mineral oil about 5 to 15% by weight of finely divided silica. The silica is dispersed together with 0.25% to 2.25% by weight of an oil-soluble acid amide of the formula



16 where  $R_1$ ,  $R_2$ , and  $R_3$  are of the group consisting of hydrogen and  $C_1-C_{24}$  aliphatic and aromatic hydrocarbon radicals (and derivatives thereof containing relatively inert functional substituents) and at least one of the substituent groups,  $R_1$ ,  $R_2$ , and  $R_3$ , is a hydrocarbon radical. In the case of acid amides in which the R group is small, the amides are water-soluble and it is necessary to include about 5 to 15% by weight of the silica of a poly-alkylene glycol waterproofing agent, such as UCON 20 25 LB 550 X, a polyalkylene glycol produced by reaction of butanol and 1,2-propylene oxide of high molecular weight (e.g., about 1400). When the R groups are sufficiently large, the acid amides are water-insoluble, as well 30 as being oil-soluble, and function as waterproofing agents for the silica particles as well as dispersants therefor.

for the silica particles as well as dispersants for the oil droplets.

Examples of acid amides which are useful as dispersants for silica-thickened grease are: N-methyl formamide, N,N-dimethyl formamide, N,N-diethyl formamide, N,N-dihexyl formamide, N,N-dihexadecyl formamide, N,N-diphenyl formamide, N,N-ditolyl formamide, N,N-dibenzyl formamide, N-butylacetamide, N-methyl acetamide, N,N-dimethyl acetamide, N,N-dibutyl acetamide, N,N-diethyl acetamide, N-hexadecylacetamide, N-methyl lactamide, N,N-dimethyl lactamide, N-butyl-lactamide, N,N-diethyl lactamide, N-methyl hexanamide, N,N-dimethyl hexanamide, N-butyl hexanamide, N,N-dibutyl hexanamide, N-phenyl hexanamide, N,N-diphenyl hexanamide, N-methyl benzamide, N,N-dimethyl benzamide, N-butyl benzamide, N,N-diphenyl benzamide, N-methyl toluamide, N,N-dibutyl toluamide, N-phenyl toluamide, N,N-phenylmethyl toluamide, butyramide, hexanamide, octanamide, octadecanamide, benzamide, toluamide, and N-octylbenzamide. These acid amides are generally operative as dispersants for silica thickened grease when added to the grease composition at a concentration of about 0.25 to 2.25% by weight of the grease.

In order to demonstrate the invention, several grease compositions were prepared to provide a comparison between the improved grease of this invention and other grease compositions.

### EXAMPLE I

60 A conventional grease-making kettle was charged with 91.2 parts by weight of 160 vis. bright stock and 0.8 part by weight of N-methyl acetamide. The mixture was thoroughly agitated and heated to 190°-215° F. To this mixture there was added 8.0 parts by weight of finely divided, amorphous silica. The silica used was "Cab-O-  
65 Sil" silica which is produced by the high-temperature reaction of a siliceous material, e.g., high-temperature, vapor-phase hydrolysis of silicon tetrachloride. The agitation of the mixture was continued during addition of the silica gelling agent and the mixture was further agi-  
70 tated and maintained at 190°-215° F. for a period of about 90 minutes. The grease thus produced was then charged to a colloid mill with a rotor-stator clearance

of 0.003", and was milled at a flow rate of 0.6-0.7 pound per minute. The grease thus obtained was then allowed to cool and was tested using a standard cone-penetration test. The grease had an unworked penetration of 232 and a worked penetration of 239, which is a NLGI #3 grease. The narrow range between unworked and worked penetrations is indicative of a high shear stability in this grease. This grease is limited to essentially anhydrous applications since it is decomposed by contact with large amounts of water. The grease, however, can be rendered stable to water by incorporation therein, during the initial agitation step, of a suitable waterproofing agent, such as Ucon LB550X (a polyethylene glycol waterproofing agent, previously identified), in the same amount as the acid amide.

#### EXAMPLE II

To a conventional grease-processing kettle there was charged a mixture of 91.2 parts by weight of 160 vis. bright stock and 0.8 part by weight of N-methyl lactamide. The mixture was thoroughly agitated and heated to 190°-215° F. To this mixture there was added 8.0 parts by weight of finely divided "Cab-O-Sil" silica. The agitation of the mixture was continued during the addition of the silica, and the mixture was agitated and maintained at 190°-215° F. for a period of about 90 minutes. The grease was then charged to a colloid mill with a rotor-stator clearance of 0.003", and was milled at a flow rate of 0.6-0.7 pound per minute. The grease was then allowed to cool and was tested using a standard cone-penetration test. This grease had an unworked penetration of 251 and a worked penetration of 263, corresponding to a #2 grease. The narrow range of the worked and unworked penetration indicates a high shear stability for this grease. This grease also is limited in application to substantially anhydrous conditions unless a waterproofing agent (Ucon LB550X, in the same proportion as the N-methyl lactamide) is used. When the grease is waterproofed, as just described, there is no appreciable change in yield or hardness.

#### EXAMPLE III

In still another experiment a grease was compounded, using the procedure described in Examples I and II, from 90.08 parts by weight of 160 vis. bright stock, 0.92 part by weight of Ucon LB550X (a polyalkylene glycol produced by reaction of butanol and 1,2-propylene oxide and having an average molecular weight of about 1400), and 9.0 parts by weight of "Cab-O-Sil" silica. The grease produced from these ingredients had an unworked penetration of 241 and a worked penetration of 275, a #2 grease. The wide range between the unworked and worked penetration in this grease, however, is indicative of relatively poor shear stability. Furthermore, the higher percentage of silica required for this grease is indicative of a much lower yield of the grease, relative to the greases produced in Examples I and II.

#### EXAMPLE IV

In several other experiments greases were compounded, using the procedure of Examples I and II, having the compositions and consistencies indicated in Table I:

Table I

| Grease No.                         | 4    | 5    | 6    | 7    | 8    | 9    | 10   |
|------------------------------------|------|------|------|------|------|------|------|
| Composition—Parts by Wt.:          |      |      |      |      |      |      |      |
| 160 vis. Bright Stock              | 91.2 | 91.2 | 91.2 | 91.2 | 91.2 | 91.2 | 91.2 |
| Silica <sup>1</sup>                | 8.0  | 8.0  | 8.0  | 8.0  | 8.0  | 8.0  | 8.0  |
| Acid Amide Dispersant <sup>2</sup> | 0.8  | 0.8  | 0.8  | 0.8  | 0.8  | 0.8  | 0.8  |
| Consistency:                       |      |      |      |      |      |      |      |
| Unworked Penetration               | 223  | 248  | 250  | 288  | 232  | 245  | 250  |
| Worked Penetration                 | 236  | 258  | 260  | 291  | 242  | 256  | 268  |

<sup>1</sup> "Cab-O-Sil" Silica.

<sup>2</sup> Grease No. 4—N,N-dimethyl formamide. Grease No. 5—N-butyl acetamide. Grease No. 6—N,N-dibutyl acetamide. Grease No. 7—N-hexadecyl acetamide. Grease No. 8—butyramide. Grease No. 9—hexanamide. Grease No. 10—N,N-diphenyl formamide.

While there have been described several preferred embodiments of this invention, including several specific examples of the best mode of carrying out this invention, it should be understood that within the scope of the appended claims this invention may be practiced otherwise than as specifically described.

What is claimed is:

1. A lubricating grease consisting essentially of a major portion of a petroleum lubricating oil having incorporated therein sufficient finely divided silica to produce a gel-like grease structure and an oil-soluble acid amide of the formula



where R<sub>1</sub>, R<sub>2</sub>, and R<sub>3</sub> are of the group consisting of hydrogen and C<sub>1</sub>-C<sub>24</sub> hydrocarbon radicals and at least one of the substituents R<sub>1</sub>, R<sub>2</sub>, and R<sub>3</sub> is a hydrocarbon radical, in an amount sufficient to effect the complete dispersion of the silica.

2. A lubricating grease according to claim 1 in which the acid amide is present in the amount of 0.25 to 2.25% by weight of the grease.

3. A lubricating grease according to claim 1 in which the silica used in an amorphous silica of very fine particle size produced by the high-temperature, vapor-phase reaction of a siliceous material.

4. A lubricating grease according to claim 1 which additionally includes 5 to 15% by weight of the silica of a waterproofing agent for the silica.

5. A lubricating grease according to claim 1 in which the acid amide is of the group consisting of N-substituted formamides, N-substituted acetamides, N-substituted lactamides, butyramide, and hexanamide.

6. A lubricating grease according to claim 4 in which the waterproofing agent is a polyoxyethylene glycol.

7. A lubricating grease consisting essentially of a major portion of a petroleum lubricating oil having incorporated therein 5-20% by weight of an amorphous silica of very fine particle size, produced by high-temperature reaction of a siliceous compound, and 0.25 to 2.25% by weight of the grease of a dispersing agent for the silica consisting of an oil-soluble hydrocarbon-substituted acid amide of the formula



where R<sub>1</sub>, R<sub>2</sub>, and R<sub>3</sub> are of the group consisting of hydrogen and C<sub>1</sub>-C<sub>24</sub> hydrocarbon radicals and at least one of the substituents R<sub>1</sub>, R<sub>2</sub>, and R<sub>3</sub> is a hydrocarbon radical.

8. A lubricating grease according to claim 7 which additionally includes 5-15% by weight of the silica of a polyoxyethylene glycol waterproofing agent for the silica.

9. A lubricating grease according to claim 7 in which the acid amide is an N-substituted formamide.

10. A lubricating grease according to claim 7 in which the acid amide is an N-substituted acetamide.

11. A lubricating grease according to claim 7 in which the acid amide is an N-substituted lactamide.

12. A lubricating grease according to claim 7 in which the acid amide is hexanamide.

13. A lubricating grease according to claim 7 in which the acid amide is butyramide.

14. A lubricating grease according to claim 7 in which the acid amide is an N-methyl acetamide.

15. A lubricating grease according to claim 7 in which the acid is N-methyl lactamide.

16. A lubricating grease according to claim 7 in which the acid amide is N,N-dimethyl formamide.

17. A lubricating grease according to claim 7 in which the acid amide is N,N-diphenyl formamide.

18. A lubricating grease according to claim 7 in which the acid amide is N-butyl acetamide.

19. A lubricating grease according to claim 7 in which the acid amide is N,N-dibutyl acetamide.

20. A lubricating grease according to claim 7 in which the acid amide is N-hexadecyl acetamide.

## References Cited in the file of this patent

## UNITED STATES PATENTS

|           |          |               |
|-----------|----------|---------------|
| 2,636,028 | Sommer   | Apr. 21, 1953 |
| 2,640,822 | Harman   | June 2, 1953  |
| 2,746,922 | Braendle | May 22, 1956  |
| 2,766,205 | Marshall | Oct. 9, 1956  |